

Feb. 10, 1959

R. H. BAILES ET AL

2,873,165

Filed May 26, 1950

## URANIUM RECOVERY PROCESS

3 Sheets-Sheet 1



*INVENTORS.*  
RICHARD H. BAILES  
ROBERT S. OLSON  
HERBERT O. KERLINGER  
RAY S. LONG

BY RAY S. LONG

Roland G. Anderson

*ATTORNEY.*

Feb. 10, 1959

R. H. BAILES ET AL  
URANIUM RECOVERY PROCESS

2,873,165

Filed May 26, 1950

3 Sheets-Sheet 2



Fig. 2.

INVENTORS.  
RICHARD H. BAILES  
ROBERT S. OLSON  
HERBERT O. KERLINGER  
RAY S. LONG  
BY

*Roland A. Anderson*

ATTORNEY.

Feb. 10, 1959

R. H. BAILES ET AL

2,873,165

URANIUM RECOVERY PROCESS

Filed May 26, 1950

3 Sheets-Sheet 3



Fig. 3.

INVENTORS.  
RICHARD H. BAILES  
ROBERT S. OLSON  
HERBERT O. KERLINGER  
RAY S. LONG

BY

*Roland A. Anderson*

ATTORNEY.

1

2,873,165

## URANIUM RECOVERY PROCESS

Richard H. Bailes, Walnut Creek, Ray S. Long, Vallejo, Robert S. Olson, San Francisco, and Herbert O. Kerlinger, Berkeley, Calif., assignors, by mesne assignments, to the United States of America as represented by the United States Atomic Energy Commission

Application May 26, 1959, Serial No. 164,566

14 Claims. (Cl. 23—14.5)

This invention relates to processes for recovering uranium from solutions and, more particularly, relates to the recovery of uranium from phosphoric acid or other phosphatic solutions.

The presence of low concentrations of uranium in certain phosphatic ores has been known for some time but the direct recovery of uranium from this source has not been economically feasible due to the low concentration of uranium present. Since these ores are presently utilized in the preparation of superphosphate and phosphoric acid in processes wherein sulfuric acid is employed for leaching the phosphatic materials from the ore and wherein the uranium is leached into the resulting acidic phosphatic solutions, there exists a possibility of recovering this low grade uranium from the solutions which are processed. However, the recovery of uranium from the phosphatic solution is complicated both by the low concentration thereof and the high concentration of phosphate in the solution in which solution the uranium is highly soluble due to complexing phenomena.

Now it has been found that low concentrations of uranium may be recovered from crude phosphoric acid or other acidic phosphatic solutions by reducing the uranium to the tetravalent state and precipitating the uranium as a fluoride and, further, that the uranium may be recovered from the precipitate by the various methods more fully described hereinafter.

Accordingly, it is an object of the invention to provide a method for recovering uranium from phosphoric acid or other phosphatic solutions.

Another object of the invention is to provide a fluoride precipitation method for recovering uranium from phosphoric acid or other phosphatic solutions.

A further object of the invention is to provide uranium recovery processes wherein a fluoride precipitate containing uranium is defluorinated and the uranium is recovered from the defluorinated precipitate.

A still further object of the invention is to provide uranium recovery processes wherein uranium is leached from a fluoride precipitate and the uranium is recovered from the leach solution.

Other objects and advantages of the invention will become apparent from the following description taken in conjunction with the accompanying drawing of which:

Figure 1 is a flow sheet of the processes of the invention;

Fig. 2 is a graphical illustration of the dependence of uranium recovery upon precipitant ratios and amounts; and

Fig. 3 is a graphical illustration of the dependence of the leaching characteristics of defluorinated and calcined fluoride precipitates upon time and temperature of calcination.

Relatively concentrated phosphoric acid or phosphatic solutions containing uranium in low concentrations such as are obtained in various phosphate fertilizer and metallurgical processes as by-products, intermediate products

2

or as final products are suitable for processing by the method of the invention.

Illustratively, such a solution may have the composition indicated in the following table:

| Table 1                        |         |       |
|--------------------------------|---------|-------|
| U <sub>3</sub> O <sub>8</sub>  | mg./l.  | 105   |
| H <sub>3</sub> PO <sub>4</sub> | g./l.   | 330   |
| V                              | g./l.   | 1.40  |
| Fe                             | g./l.   | 3.02  |
| 10 Cu                          | percent | 0.155 |
| Mg                             | do      | 0.20  |
| Al                             | do      | 0.34  |
| F                              | do      | 1.13  |
| 15 Sulfate                     | do      | 1.22  |
| Sp. Gr.                        |         | 1.207 |

However, solutions differing very considerably from that indicated either in relative concentrations or in the types of ions present may also be satisfactorily processed.

20 With reference to the flowsheet of Fig. 1, and in accordance with the invention a phosphate or phosphoric acid solution of the character described is subjected to reduction, whereby all of the uranium contained therein is reduced to the tetravalent state. The reduction of the uranium to the tetravalent state may be accomplished utilizing metallic reducing agents such as iron, zinc, zinc amalgam, aluminum or lead, or by using reducing agents such as hydrazine salts, hypophosphorous acid or hydroxylamine hydrochloride or by electrolytic methods. The requirements for the reducing agent are not critical and a majority of the reducing agents having a sufficiently high reducing potential appear to be suitable for the purpose. The progress of the reduction is easily followed by observing the electromotive potential developed between platinum and saturated calomel electrodes immersed in the solution. Reduction is substantially complete when the potential is lowered to about +0.1 volt.

Following reduction, the solution is treated to coprecipitate the reduced uranium as a fluoride together with other insoluble fluorides thereby achieving a substantially complete removal of even very small quantities of uranium from the phosphatic solution. In the event that the solution is deficient in coprecipitant materials, a sufficient quantity of a soluble compound of

45 the coprecipitant is supplied to the solution and then a soluble fluoride or hydrofluoric acid is added to coprecipitate the reduced uranium with the coprecipitant material. Calcium carbonate, calcium oxide, hydrated calcium oxide, and barium carbonate have been found satisfactory to supply the required coprecipitant materials; however, other materials may also be used as will become apparent from the following discussion. Various soluble fluorides, such as sodium fluoride, potassium fluoride, barium fluoride and ammonium fluoride and other fluorides which furnish a considerable fluoride ion concentration to the solution, may be employed in the precipitation, also hydrofluoric acid (hydrogen fluoride) is completely satisfactory. The ratio of cation equivalents to fluoride equivalents present in the acid and the total amount of precipitants present determine to a critical degree the amount of uranium which is recovered in the precipitate. Fig. 2 graphically illustrates the close and critical relationship which these factors bear to the amount of uranium recovered.

55 60 65 The mechanism of the precipitation of uranium from the phosphoric acid solution is not completely understood. It has been noted that the presence of aluminum in the solution greatly increases the recovery of uranium. In the presence of aluminum a cryolite type of compound precipitates which compound is preferentially precipitated rather than uranous fluoride. The cryolite

70

compound which precipitates appears to have the general formula  $X(\text{AlF}_6)_n$  wherein  $X$  may represent various proportions and combinations of radicals such as uranous uranium, Mg, Ca, Na, K,  $\text{NH}_4$  and others. The existence of compounds such as  $\text{Mg}_2(\text{AlF}_6)_2$  and  $\text{Ca}_3(\text{AlF}_6)_2$  in the precipitate has been indicated by X-ray diffraction studies. Moreover, a mixture of various other insoluble fluorides may be precipitated along with the insoluble uranium compound. Some of the fluoride originally present in the acid and that added during the precipitation may be recovered from the precipitate and from the solution for recycling by methods more fully described hereinafter.

The fluoride precipitate containing uranium is separated from the solution by filtering and the uranium is recovered from the precipitate by one of several alternative methods and the filtrate is treated for recovery of the fluoride or/and is returned to the plant for normal processing.

A typical precipitate derived from such a solution using calcium carbonate and hydrogen fluoride as the precipitants may have a composition determined by analysis approximately as follows: However, it will be appreciated that the composition of such a precipitate may vary considerably from that indicated dependent upon the composition of the original acid and conditions of precipitation.

|                        | Percent |
|------------------------|---------|
| $\text{U}_3\text{O}_8$ | 0.25    |
| Phosphate              | 1.95    |
| Sulfate                | 0.85    |
| Ca                     | 19.55   |
| Al                     | 8.6     |
| Mg                     | 4.95    |
| F                      | 47.0    |

Emission spectrographic analysis discloses that other materials may be present as follows:

|    | Percent    |
|----|------------|
| Fe | 0.5-1.0    |
| Na | 0.5-1.0    |
| Si | 0.05-0.10  |
| V  | 0.05-0.10  |
| Cu | 0.001-0.01 |
| Cr | 0.001-0.01 |
| Mn | 0.001-0.01 |
| Ti | 0.001-0.01 |

In general the methods of uranium recovery which are employed may be classed in two groups; one, in which the uranium is recovered from the precipitate following defluorination of the precipitate; or, two, in which the uranium is recovered from the precipitate prior to defluorination.

In the methods of the first classification, sulfuric acid is added to the precipitate in stoichiometric excess relative to the quantity of fluoride present and hydrogen fluoride is vaporized from the precipitate and recovered in order that it may be recycled. Alternatively, ammonium sulfate is added to the precipitate and ammonium fluoride is sublimed from the precipitate and recovered for recycling. Then the defluorinated precipitate is calcined and leached with water or a solution such as dilute hydrochloric, nitric or sulfuric acid solutions and the uranium is finally recovered from the leach solution.

The temperature to which the precipitate is heated in driving off the fluoride affects the conditions which must be employed during the leaching. If the precipitate, following treatment with sulfuric acid, is heated to a temperature below about  $800^\circ \text{C}$ , for  $1\frac{1}{2}$  to 2 hours the precipitate produces an acidic solution on contact with water since aluminum sulfate appears to be formed by this treatment which aluminum sulfate produces a sufficiently acid solution to extract the uranium. However, if the heating time is prolonged or the temperature is increased to about  $800$ – $1000^\circ \text{C}$ , alkaline products pre-

5 dominate in the heated precipitate and an acidic solution must be employed to leach the uranium. Moreover, the solubility of various components of the precipitate is markedly affected by the time and temperature of heating; little aluminum and/or magnesium being leached from the more intensively heated materials.

10 The composition of a leach liquor typical of those which are derived by leaching a fluoride precipitate, which was heated to a temperature of  $800$  to  $1000^\circ \text{C}$ , for  $1\frac{1}{2}$  to 3 hours with a slight excess of sulfuric acid, employing 1% sulfuric acid is indicated below in Table 2. About 80–90% of the uranium, none of the aluminum, and only one-third of the magnesium was leached.

Table 2

|                        | Grams/liter |
|------------------------|-------------|
| $\text{U}_3\text{O}_8$ | 0.6         |
| Ca                     | 0.4         |
| Mg                     | 3           |
| Al                     | 0.0         |
| Phosphate              | 8           |
| Sulphate               | 35          |
| V                      | 0.2         |

25 The variations in leach liquor characteristics with variation in time and temperature of defluorination-calcination and leach reagent are graphically indicated in Fig. 3. The time-temperature curve (A) of defluorination are plotted with respect to the leach liquor pH (reading upwards) curve (B); percentage of uranium leached, curve (C); percentage of aluminum leached, curve (D); and percentage of Mg leached, curve (E).

30 Optimum conditions for a sulfuric acid leach are as follows: 0.2 N or about 1% sulfuric acid as the leach reagent; minus 40 mesh size of the precipitate; and a liquid to solid ratio of about 2.5:1.

The uranium may be recovered from the leach liquor by two methods:

(1) Precipitation of uranyl phosphate by pH adjustment, yielding 99.9% uranium recoveries of a material which after ignition contains uranium equivalent to about 10%  $\text{U}_3\text{O}_8$ , employing amounts of sodium hydroxide equivalent to about 8 to 16 grams per gram of  $\text{U}_3\text{O}_8$  precipitated.

(2) By reduction of the leach liquor with sodium hydrosulfite, or other suitable reducing agents, 99+-% of the uranium is precipitated in a material containing about 10 to 20%  $\text{U}_3\text{O}_8$ . An analysis of a typical precipitate of this type follows:

|                        | Percent |
|------------------------|---------|
| $\text{U}_3\text{O}_8$ | 13.8    |
| Phosphate              | 30.3    |
| Sulfate                | 1.5     |
| Ca                     | 3.1     |
| Al                     | 11.6    |
| Mg                     | 1.1     |

55 In the methods of the second classification, hot sodium carbonate is employed to leach the uranium from the fluoride precipitate with great efficiency while ammonium carbonate may also be employed if somewhat less leaching efficiency can be tolerated. The leaching efficiency of sodium carbonate solutions drops off very rapidly below a critical pH value between about 8.5 and 9.0. A decrease in efficiency is noted with increasing solid to liquid ratios and a marked increase if the temperature at which the leaching is performed is increased to near the boiling point. Carbonate leaches all of the sulfate; about 0.1% of the phosphate, 0.8% of the aluminum and 2% of the fluoride from the precipitate in addition to the uranium.

60 Uranium contained in the leach solutions is in the uranyl state due to oxidation by air or by the various treatments. The uranium may be recovered from the sodium carbonate leach solution preferably by neutralizing the solution with hydrochloric acid and precipitating the uranium in a purified form with carbonate-free

ammonia as ammonium diuranate. If there is present a considerable concentration of phosphate in the solution, uranyl phosphate or a mixture of uranyl phosphate and ammonium diuranate is precipitated. Precipitated ammonium diuranate is then calcined to yield high grade  $U_3O_8$ . The leached precipitate may then be treated to recover the fluorine or is discarded.

Alternatively, in the second classification of methods, acidic leaching of the fluoride precipitate may be employed without washing the precipitate. Dilute aqueous solutions of hydrochloric, nitric, citric acid and less effectively tartaric, acetic and boric acids are used to leach the uranium from the precipitate with the uranium concentration being enhanced by successively leaching several portions of precipitate with the same solution and uranium is recovered from the acid leach solution by precipitation methods which further increase the purity of the material.

Acid leaching of the precipitate has been found to be influenced by the following variables as exemplified when dilute hydrochloric acid is employed; concentration of acid, time of leaching, temperature, solid to liquid ratio and phosphate concentration in the fluoride precipitate. Optimum conditions for leaching more than 95% of the uranium from a dry fluoride precipitate require a 30 to 35 minute leach with agitation at 95° C. with 5 to 10 ml. of 5% hydrochloric acid per gram of fluoride precipitate. Lowering the leaching temperature to 25° C. decreases the uranium recovery to 75% and a five minute leach yields only 30% uranium recovery. Leach times beyond 30 minutes show no improvement in uranium recovery. When acid concentrations above about 5% are employed the loss of fluoride from the precipitate becomes large and lower concentrations decrease the uranium recovery. Markedly decreased uranium recovery is noted with lower solid to liquid ratios while higher liquid to solid ratios show only a slight improvement.

Reduction of the uranium in the leach solution with various reducing agents causes the formation of a uranous phosphate precipitate with the phosphate which is leached into the hydrochloric acid solution. Sodium hydrosulfite, added to the solution as a reductant, precipitates a material containing uranium equivalent to about 55 to 65%  $U_3O_8$  and about 30% of phosphate.

Particular details of the processes of the invention will become apparent from a consideration of the following illustrative examples of the operation of processes in accordance with the invention:

#### EXAMPLE A

17.1 liters of a solution having the composition indicated in Table I was reduced by contact with metallic iron to a potential of +0.08 V. as measured with a platinum-standard calomel electrode system.

Table I

|           |         |       |
|-----------|---------|-------|
| $H_3PO_4$ | g./l.   | 307   |
| $U_3O_8$  | mg./l.  | 110   |
| V         | g./l.   | 1.32  |
| Fe        | g./l.   | 3.10  |
| Ca        | percent | 0.13  |
| Mg        | do      | 0.19  |
| Al        | do      | 0.29  |
| F         | do      | 1.16  |
| Sulfate   | do      | 1.52  |
| Sp. Gr.   |         | 1.205 |

24.7 grams per liter of calcium carbonate and 25 grams per liter of aqueous hydrogen fluoride added to the solution produced a precipitate weighing 694 grams, substantially free of phosphate after washing, and containing 0.21% uranium and about 78% of the recoverable fluorine. This uranium recovery amounts to about 94% based on the uranium content of the various precipitates and filtrates.

Portions of the precipitate were defluorinated by adding an excess of concentrated sulfuric acid and heating the mixture for 130 minutes to a maximum temperature of 900° C. 130 grams of this defluorinated material was leached with 325 cc. of 0.2 N sulfuric acid at a temperature of 90° C. for 15 minutes with a resultant removal of 68% of the uranium by the leach liquor. A second leaching of the same material with 325 cc. of 0.4 N sulfuric acid for 30 minutes at 95° C. raised the overall amount of uranium leached by the two successive operations to 98% of the uranium originally present in the material being treated.

#### EXAMPLE B

15 Phosphoric acid having the composition indicated in Table II was used in this experiment.

Table II

|    |           |           |      |
|----|-----------|-----------|------|
| 20 | $H_3PO_4$ | percent   | 30.2 |
| 20 | $U_3O_8$  | mg./liter | 104  |
| 20 | Al        | percent   | 0.29 |
| 20 | Mg        | do        | 0.23 |
| 20 | Ca        | do        | 0.11 |
| 25 | Sulfate   | do        | 1.75 |
| 25 | V         | g./liter  | 1.5  |
| 25 | Fe        | g./liter  | 3.1  |
| 25 | Sp. Gr.   |           | 1.21 |

20.7 liters of this acid was reduced by circulation through a metallic iron packed column until the electro-motive potential of the solution as measured between platinum and standard calomel electrodes was +0.033 V. The reduced solution was then treated with 360 g. of calcium carbonate and 476 g. of fluorine as an aqueous solution of HF to precipitate the uranium. After washing with water and drying at 120° C. for 24 hours the precipitate weighed 805 g. and had the composition indicated in Table III.

Table III

|    |           |         |       |
|----|-----------|---------|-------|
| 40 | $U_3O_8$  | Percent | 0.177 |
| 40 | Ca        | 15.9    |       |
| 40 | Mg        | 3.6     |       |
| 40 | Al        | 10.6    |       |
| 45 | Phosphate | 3.9     |       |
| 45 | F         | 48.5    |       |
| 45 | V         | 0.043   |       |
| 45 | Sulfate   | 1.55    |       |

This percentage of uranium amounts to a recovery of 76% of the uranium originally present in the acid and is slightly lower than that normally obtained due to incomplete reduction of the acid. Portions of this precipitate were defluorinated and calcined by heating with concentrated sulfuric acid using the conditions indicated in Table IV. Portions of these defluorinated materials were then leached employing the conditions indicated under the appropriate heading of Table IV. The water and 0.092 N sulfuric acid leach being done on the material heated for 100 minutes at 800° C. and the 0.18 N sulfuric acid leach being done on the material heated for 170 minutes at 900° C.

Table IV

#### DEFLUORINATION

|    |                                   |     |     |
|----|-----------------------------------|-----|-----|
| 65 | $H_2SO_4$ percent excess          | 6.9 | 5   |
| 65 | Defluorination time, min.         | 100 | 170 |
| 65 | Max. Temp. of defluorination, °C. | 800 | 900 |

#### LEACH

70 [50 g. of defluorinated material leached with 125 cc. of reagent.]

|                             |         |           |           |
|-----------------------------|---------|-----------|-----------|
| Leach reagent               | $H_2O$  | $H_2SO_4$ | $H_2SO_4$ |
| Concentration of reagent    | 0.092 N | 0.18 N    |           |
| Identification leach liquor | A       | B         | O         |
| U leached, percent          | 85      | 94        | 87        |

Uranium contained in these leach liquors was recovered by treating 25 ml. portions with 0.5 g. of sodium hydrosulfite resulting in the precipitation of 81 and 99.9%, respectively, of the uranium from leach liquors A and C as a precipitate containing 13.4 and 19.1% of U.

Also, the uranium was recovered as uranyl phosphate by adding alkali to the solutions. 25 ml. of leach solution B was treated with 26 ml. of 0.1 N NaOH resulting in the precipitation of 41% of the uranium present in a precipitate containing 5.1% U. 25 ml. portions of solution C were treated with 18.8 and 39.2 ml. of 0.1 N NaOH, respectively, resulting in the precipitation of 99.7 and 99.9% of the uranium in a precipitate containing 10.3 and 9.7% U.

### EXAMPLE C

2 liters of 35% commercial phosphoric acid containing 108 mg./liter of  $U_3O_8$  was reduced with iron and the uranium precipitated by the addition of 36 g. of calcium carbonate and 52.8 g. of hydrogen fluoride. About 90% of the uranium was found in the precipitate. This precipitate containing 190 mg. of  $U_3O_8$  was successively leached with sodium carbonate solution as follows:

|                       | Extracted                                    |
|-----------------------|----------------------------------------------|
| Solution:             |                                              |
| A                     | 30 g. $Na_2CO_3$ in 500 ml. $H_2O$ at 25° C. |
| B                     | 40 g. $Na_2CO_3$ in 500 ml. $H_2O$ at 80° C. |
| C                     | 25 g. $Na_2CO_3$ in 500 ml. $H_2O$ at 80° C. |
| D                     | 25 g. $Na_2CO_3$ in 500 ml. $H_2O$ at 80° C. |
| Total (mg. $U_3O_8$ ) | 177.5                                        |

120.7 g. of the solid remaining after leaching had the following composition:

|          | Percent |
|----------|---------|
| $U_3O_8$ | 0.00015 |
| F        | 30.3    |
| $PO_4$   | 18.5    |
| $CO_3$   | 7.5     |
| Ca       | 11.9    |
| Al       | 7.5     |
| Mg       | 4.95    |
| Fe       | 0.7     |
| Na       | 17.0    |

The four solutions obtained from above were then employed in succession to leach a second similar precipitate weighing 68 g. and containing 136 mg.  $U_3O_8$  by heating for 20 min. at 80° C. with the following results.

|   | $U_3O_8$ Content of Leaching Solution, mg. | $U_3O_8$ Content After Leaching, mg. |
|---|--------------------------------------------|--------------------------------------|
| A | 3.6                                        | 0.4                                  |
| B | 69.0                                       | 157.0                                |
| C | 68.4                                       | 121.0                                |
| D | 36.5                                       | 40.0                                 |
|   | 177.5                                      | 318.4                                |

In the same manner another precipitate was treated with these four solutions resulting in the  $U_3O_8$  content of the combined solutions being raised to 500 mg. The combined solutions were heated with hydrochloric acid to remove the carbonate and ammonia was added to precipitate the uranium. There was obtained a precipitate weighing 0.7338 g. which contained 66.3%  $U_3O_8$ , 23.8%  $PO_4$ , 9.7%  $SiO_2$ , and 0.55% vanadium, thus indicating that the product was fairly pure uranyl phosphate.

### EXAMPLE D

Both leached (with  $Na_2CO_3$ ) and unleached precipitated material was defluorinated by heating with ammonium sulphate and sulfuric acid as indicated in Table V.

8  
Table V

| Wt. of ppt. g.     | Fluorine Content, percent | $(NH_4)_2SO_4$ used, g. | Time and Temp. of heating | Fluoride sublimed, percent |
|--------------------|---------------------------|-------------------------|---------------------------|----------------------------|
| 9.96 <sup>1</sup>  | 30.3                      | 10.02                   | 24 hr./450° C.            | 83.2                       |
| 5.00 <sup>2</sup>  | 49.2                      | 8.20                    | 1.5 hr./450° C.           | 97.1                       |
| 10.00 <sup>2</sup> | 49.2                      | 16.00                   | 1.5 hr./450° C.           | 97.9                       |
| 10.00 <sup>2</sup> | 44.9                      | 20.00                   | 1.5 hr./450° C.           | 99.1                       |
| 15.00 <sup>2</sup> | 44.9                      | 10.01                   | 1.5 hr./450° C.           | 98.9                       |
| 10.48 <sup>2</sup> | 44.9                      | 8.01                    | 1.5 hr./450° C.           | 98.5                       |
| 5.06 <sup>2</sup>  | 44.9                      | 16.00                   | 1.5 hr./450° C.           | 98.8                       |
| 5.04 <sup>2</sup>  | 44.9                      | 18.00                   | 1.5 hr./450° C.           | 99.0                       |
| 7.05 <sup>2</sup>  | 44.9                      | 3.83                    | 1.5 hr./450° C.           | 70.8                       |
| 5.01 <sup>2</sup>  | 44.9                      | 6.02                    | 1.5 hr./450° C.           | 90.1                       |
| $H_2SO_4$          |                           |                         |                           |                            |
| 100 <sup>3</sup>   | 46.7                      | 135                     | 1/4 hr./875° C.           | 97.1                       |
| 100 <sup>2</sup>   | 46.7                      | 135                     | 1/2 hr./700° C.           | 99.0                       |
| 100 <sup>2</sup>   | 46.7                      | 135                     | 1/4 hr./500° C.           | 94.4                       |

<sup>1</sup> Leached.  
<sup>2</sup> Unleached.

### EXAMPLE E

Various reducing agents were employed to reduce two liter portions of industrial (35%) phosphoric acid containing 108 mg.  $U_3O_8$ /liter and the uranium was precipitated under the conditions and with the results indicated in Table VI.

Table VI

| Reducing Agent | Precipitating Agents | ppt. Wt., g. | $U_3O_8$ in ppt., percent | Recovery of $U_3O_8$ from acid, percent |
|----------------|----------------------|--------------|---------------------------|-----------------------------------------|
| (1) Pb         | 45 g. $NH_3$         | 46.3         | 0.166                     | 50                                      |
|                | 52.9 g. HF           |              |                           |                                         |
|                | 36 g. $CaCO_3$       | 86.7         | 0.14                      | 72                                      |
|                | 52.8 g. HF           |              |                           |                                         |
|                | 20 g. $CaO$          | 69.2         | 0.16                      | 70                                      |
|                | 45 g. HF             |              |                           |                                         |
|                | 20 g. $CaO$          | 69.1         | 0.29                      | 92.5                                    |
|                | 45 g. $NH_3$         | 47.0         | 0.22                      | 71                                      |
|                | 52.8 g. HF           |              |                           |                                         |
|                | 20 g. $CaO$          | 91.6         | 0.23                      | 91                                      |
|                | 52.8 g. HF           |              |                           |                                         |
|                | 10 g. $CaO$          | 53.7         | 0.19                      | 54                                      |
| (2) Pb         | 52.8 g. HF           |              |                           |                                         |
|                | 20 g. $CaO$          | 92.5         | 0.21                      | 94                                      |
|                | 52.8 g. HF           |              |                           |                                         |
|                | 20 g. $CaO$          | 82           | 0.22                      | 87                                      |
|                | 52.8 g. HF           |              |                           |                                         |
|                | 20 g. $CaO$          |              |                           | 98                                      |
|                | 52.8 g. HF           |              |                           |                                         |
|                | 20 g. $CaO$          |              |                           | 93                                      |
|                | 52.8 g. HF           |              |                           |                                         |
|                | 3.6 g. $CaO$         | 86           | 0.27                      | 90                                      |
|                | 52.8 g. HF           |              |                           |                                         |

Uranium was recovered from several of the precipitates listed in Table VI by the following methods:

Precipitate (9) weighing 82 g. and containing 0.22% or 180 mg. of  $U_3O_8$  was heated with 400 ml. of a solution containing 50 g. of  $Na_2CO_3$  for 2 hours with a resultant leaching of 128 mg. or 71.3% of the uranium.

Precipitate (10) a well washed precipitate weighing 187.8 g. wet which is equivalent to 53.3 g. dry and containing 0.27% or 144 mg. of  $U_3O_8$  was heated for 1 1/2 hours with 400 ml. of a solution containing 50 g.  $Na_2CO_3$  resulted in the leaching of 100% of the uranium from the precipitate. This leach solution which now amounted to 595 ml. due to wash water inclusion was then employed to leach the entire wet precipitate (11), after an additional 25 g. of  $Na_2CO_3$  was added and with heating for 1 1/2 hours. The leach filtrate contained 259 mg. of  $U_3O_8$  amounting to a 57% extraction of uranium from the second precipitate in addition to that extracted from the first.

Precipitate (12) from above was subjected to successive leachings with fresh portions of carbonate solution as follows:

(1) The entire precipitate containing 190 mg. of  $U_3O_8$  was stirred for 1 1/2 hours with a cold solution of

50 g. of  $\text{Na}_2\text{CO}_3$  in 500 ml. of water. The leach filtrate contained 3.6 mg.  $\text{U}_3\text{O}_8$ .

(2) The residual precipitate from (1) was stirred for 45 minutes with heating with a solution of 40 g. of  $\text{Na}_2\text{CO}_3$  in 500 ml. of water and the precipitate was separated from the solution by filtering. This filtrate contained 69 mg. of  $\text{U}_3\text{O}_8$ .

(3) The residual precipitate from 2, preceding, was heated with a 500 ml. of a solution containing 25 g.  $\text{Na}_2\text{CO}_3$  for 1½ hours and was then separated from the solution by filtering. The filtrate contained 68.4 mg. of  $\text{U}_3\text{O}_8$ .

(4) The residual precipitate from 3, preceding, was heated with 500 ml. of a solution containing 25 g. of  $\text{Na}_2\text{CO}_3$  for 45 minutes and then was filtered from the solution. The filtrate contained 36.5 mg. of  $\text{U}_3\text{O}_8$ .

The total uranium recovered amounted to 180.6 mg. as  $\text{U}_3\text{O}_8$  while 216 mg. was present in the original acid.

#### EXAMPLE F

A variety of reducing agents were employed to reduce 100 ml. portions of 35% commercial phosphoric acid containing 10.6 mg.  $\text{U}_3\text{O}_8$  using the conditions and with the results indicated in Table VII. The reduced uranium was then precipitated by the addition of 1 g.  $\text{CaO}$  and 2.64 g. of HF to the reduced solution while contained in a plastic beaker. In some cases HF was added with the reducing agent with a consequent improvement in the amount of uranium precipitated. Increased temperature also improves the recovery.

Table VII

| Reducing Agent       | Time, hr. | Tempera-ture, °C. | Recovery $\text{U}_3\text{O}_8$ , percent |
|----------------------|-----------|-------------------|-------------------------------------------|
| 30 g. Pb 10 mesh     |           | 95                | 81                                        |
| 10 g. Pb 10 mesh     |           | 95                | 67                                        |
| 10 g. Pb 10 mesh     | 2         | 95                | 78                                        |
| 2 g. Sn 10 mesh      | 3         | 95                | 63                                        |
| 5 g. Sn 10 mesh      | ½         | 95                | 67                                        |
| 30 g. Cu Turnings    | ½         | 95                | 64                                        |
| 10 g. Cu Turnings    | 1         | 95                | 88                                        |
| 2 g. Cu 80 mesh shot | 1         | 95                | 76                                        |
| 2 g. Cu 80 mesh shot |           | 95                | 86                                        |
| 2 g. Fe Turnings     |           | 25                | 94                                        |
| 2 g. Fe Turnings     | 2         | 95                | 83                                        |
| 5 g. Fe Turnings     | 1         | 25                | 89                                        |
| 4 g. Zn 20 mesh      | 1         | 25                | 81                                        |
| 2 g. Zn 20 mesh      | 1         | 25                | 94                                        |
| 1 g. Zn Amalgam      | 1         | 25                | 75                                        |
| 10 g. Zn Amalgam     | 4         | 25                | 89                                        |
| 5 g. Zn Amalgam      | 1         | 25                | 88                                        |
| 2 g. Zn Amalgam      | 1         | 25                | 88                                        |

<sup>1</sup> 2.47 g. HF added.

In the experiments using copper, only small amounts of copper appeared to dissolve. Zinc and zinc amalgam were effective reducing agents with only small amounts although zinc dissolved with evolution of hydrogen. Hydrogen is not evolved when lead is used.

In the foregoing, the uranium content is indicated in amounts or percentages of  $\text{U}_3\text{O}_8$ . However, it is not intended that this terminology is to be construed literally but is intended to indicate that the equivalent quantity of uranium is present in the appropriate form as indicated by context.

While there has been described in the foregoing what may be considered preferred embodiments of the invention, it is believed that various modifications may be made therein without departing from the spirit and scope of the invention and it is intended to cover all such as fall within the scope of the appended claims.

What is claimed is:

1. The method of recovering uranium values from a phosphatic solution containing impurity materials the fluorides of which are insoluble in said phosphatic solution comprising reducing the uranium to the uranous state in the solution, adding a soluble calcium coprecipitant compound to said solution, adding a soluble fluoride to said solution, whereby said coprecipitant and some of said

impurities are coprecipitated with the uranium to form a complex fluoride precipitate, leaching uranium from the complex fluoride precipitate, and recovering uranium from the leach solution.

5. The method of recovering uranium values from a crude phosphatic solution containing materials the fluorides of which are insoluble in said phosphatic solution, comprising reducing the uranium to the uranous state in the solution, adding a soluble calcium coprecipitant compound to said solution, adding a soluble fluoride to said solution, whereby said coprecipitant and the uranium are coprecipitated to form a complex fluoride precipitate, defluorinating and calcining said precipitate, leaching uranium from said defluorinated and calcined precipitate, and recovering uranium from the leach solution.

10. 3. The method of recovering uranium values from a crude phosphatic solution comprising reducing the uranium to the uranous state in the solution, adding a soluble calcium coprecipitant compound to said solution, adding a soluble fluoride to said solution whereby the uranium is coprecipitated with said coprecipitant to form a complex fluoride precipitate, leaching uranium from said complex fluoride precipitate under acidic conditions, and recovering uranium from the leach solution.

20. 4. The method of recovering uranium from an acidic phosphatic solution comprising treating said solution with an agent to reduce the uranium to the uranous state, coprecipitating said uranous uranium from the solution by adding soluble fluorides and at least one coprecipitant

25. 30 selected from the group consisting of calcium, barium, magnesium, aluminum, sodium, potassium and ammonia which form insoluble fluorides in said solution thereto, leaching uranium from said precipitate with an acid solution, whereby some phosphate is also leached, and treating said acidic solution with a reducing agent to precipitate said uranium from the leach solution as uranous phosphate.

35. 5. The process for recovering uranium from acidic phosphatic solutions comprising reducing said uranium to the uranous state in the solution, precipitating said uranous uranium from the solution by adding thereto soluble fluorides and coprecipitants selected from the group consisting of calcium, barium, magnesium, aluminum, sodium, potassium and ammonia which form insoluble fluorides in said solution, defluorinating and calcining said precipitate by heating with a material selected from the group consisting of sulfuric acid and ammonium sulfate, leaching uranium from said defluorinated and calcined precipitate with an acidic aqueous solution, and recovering uranium from said acidic leach solution.

40. 6. The method of recovering uranium from an acidic phosphatic solution comprising reducing said uranium to the uranous state in solution, precipitating said uranous uranium by adding to the solution soluble fluorides and coprecipitants selected from the group consisting of calcium, barium, magnesium, aluminum, sodium, potassium and ammonia which form insoluble fluorides in said solution, leaching uranium from said precipitate with a carbonate solution, acidifying said leach solution, and precipitating the uranium from the acidified leach solution as uranium diuranate by the addition of ammonia.

45. 7. The method of recovering uranium from a phosphatic solution comprising reducing said uranium to the uranous state in the solution, precipitating said uranous uranium by adding to said solution a soluble fluoride and coprecipitants selected from the group consisting of calcium, barium, magnesium, aluminum, sodium, potassium and ammonia which form insoluble fluorides in said solution, leaching uranium from said precipitate with an acid solution, and precipitating the uranium from said solution as uranyl phosphate by adjusting the pH of the solution with an alkaline material.

50. 8. The process as defined in claim 7, wherein said acid is a material selected from the group consisting of hydrochloric, nitric, citric, tartaric, acetic and boric acids.

9. The process of recovering uranium from an acidic phosphatic solution containing impurities including phosphate, sulfate, iron, silicon, vanadium, and titanium, comprising reducing the uranium to the uranous state in the solution, adding a soluble calcium coprecipitant compound to the solution, treating said solution with a soluble fluoride to precipitate said material and at least some of said impurities from the solution, whereby the uranium is coprecipitated with the precipitate, leaching uranium from said precipitate with a material selected from the group consisting of sodium carbonate and ammonium carbonate, acidifying the leach solution, and precipitating the uranium from the acidified solution with ammonia.

10. The process for recovering uranium from an acidic phosphatic solution containing impurities including phosphate, sulfate, iron, silicon, vanadium, and titanium, comprising reducing the uranium to the uranous state in the solution, adding a soluble calcium coprecipitant compound to the solution, treating said solution with a soluble fluoride to precipitate said material and at least some of said impurities from the solution, whereby the uranium is coprecipitated with the precipitate, defluorinating and calcining said precipitate by heating with a material selected from the group consisting of sulfuric acid and ammonium sulfate, leaching uranium from the defluorinated and calcined precipitate with a material selected from the group consisting of water, sulfuric acid and nitric acid, whereby some phosphate is also leached, and precipitating uranyl phosphate by making the solution alkaline.

11. The process for recovering uranium from an acidic phosphatic solution containing impurities including phosphate, sulfate, iron, silicon, vanadium, and titanium, comprising reducing the uranium to the uranous state in the solution, adding a soluble calcium coprecipitant compound to the solution, treating said solution with a soluble fluoride to precipitate said material and at least some of

said impurities from the solution, whereby the uranium is coprecipitated with the precipitate, defluorinating and calcining said precipitate by heating with a material selected from the group consisting of sulfuric acid and ammonium sulfate, leaching uranium from the defluorinated and calcined precipitate with a material selected from the group consisting of water, sulfuric acid and nitric acid, whereby some phosphate is also leached, and precipitating uranous phosphate from said solution by reducing the uranium to the uranous state.

12. The process for recovering uranium from an acidic phosphatic solution comprising reducing the uranium to the uranous state in solution, adding to said solution co-precipitant materials selected from the group consisting of calcium, barium, magnesium, aluminum, sodium, potassium and ammonia which form insoluble fluorides in said solution, treating said solution with soluble fluorides to precipitate said co-precipitant materials, whereby the uranium is coprecipitated therewith, leaching the uranium from the precipitate with an acidic solution, whereby some phosphate is also leached, and precipitating uranous phosphate from the solution by reducing the uranium to the uranous state.

13. The process as defined in claim 12, wherein said acidic solution which is employed to leach the precipitate is a material selected from the group consisting of hydrochloric, nitric, citric, tartaric, acetic and boric acid solutions.

14. The process as defined in claim 10, wherein said soluble fluoride is a material selected from the group consisting of sodium, potassium, barium and ammonia fluorides.

35 References Cited in the file of this patent

Mellor: Inorganic and Theoretical Chemistry, vol. 12, page 74 (1932). Publ. by Longmans, Green & Co., London.